

(No Model.)

W. H. MAXWELL.  
Insulated Telegraph Wire.

No. 243,283.

Patented June 21, 1881.



Witnesses.

R. Marshall  
J. C. Fawcett, Jr.

Inventor  
William H. Maxwell  
by his attorneys  
Bakewell & Kins

# UNITED STATES PATENT OFFICE.

WILLIAM H. MAXWELL, OF PHILLIPSBURG, ASSIGNOR OF TWO-THIRDS TO  
A. S. TOMPKINSON, OF PHILADELPHIA, PENNSYLVANIA.

## INSULATED TELEGRAPH-WIRE.

SPECIFICATION forming part of Letters Patent No. 243,283, dated June 21, 1881.

Application filed March 12, 1881. (No model.)

*To all whom it may concern:*

Be it known that I, WILLIAM H. MAXWELL, of Phillipsburg, in the county of Beaver and State of Pennsylvania, have invented a new and useful Improvement in Insulated Telegraph-Wires; and I do hereby declare the following to be a full, clear, and exact description thereof.

Heretofore metal-incased insulated wire has been made by placing a wire in a glass tube and the glass tube in a wrought-iron tube, heating the whole, and then drawing it out to the required size and length in suitable rolls. This article has been open to the objection that it is nearly if not quite impossible, in practice, to use more than one wire, and that the glass in all cases is fractured or "crizzled" by the reheating and rolling operation, and that in case of any defect or leak in the outer casing 20 admitting water or moisture the same will obtain access to the wire through the cracks or crizzles and destroy the insulation.

My invention is designed to overcome this difficulty, and is a glass-insulated telegraph wire or wires having an external casing of cast-iron.

To enable others skilled in the art to make and use my invention, I will now describe it by reference to the accompanying drawings, in 30 which—

Figure 1 is a view of my improved glass-insulated metal-incased telegraph-wire; Fig. 2, an illustration of one way of making it, and Fig. 3 another way of making it.

Like letters of reference indicate like parts in each.

My improved glass-insulated metal-incased telegraph-wire cable is shown in Fig. 1, in which *a* are the wires, which may be one or 40 more, as desired; *b*, the glass insulating layers, and *c* the cast-iron casing. This article may be produced, as shown in Fig. 2, by the use of a vertical partible or solid mold, *d*, having a flaring mouth, *d'*, and a moving bottom, *e*, and surrounded by a water-box, *f*, having water inlet, outlet, and drain-pipes *f'*, *f''*, and *f'''*. The bottom *e* is perforated vertically, as at *e'*. The wires *a* are in uniform lengths, and are fastened to the bottom *e* by passing them through the

perforations *e'*, and then twisting the ends, as at *e''*. Small glass tubes *b* are slipped on the wires, covering them completely. The bottom is lowered in the mold a short distance below the flaring mouth, and the molten cast-iron is poured in from a suitable ladle or cupola, and when it rises nearly to the top the bottom is lowered slowly and steadily in the mold as the metal continues to flow in. The lower part of the casting hardens, and in case it is desired to make the section longer than the mold the bottom may be permitted to descend below the open end of the mold. If the column is too heavy to be properly supported by the wires, additional support may be given to it from below. To prevent the metal from adhering to the mold before the bottom begins to descend, liners of sheet-iron or other suitable material may be placed inside of the mold at that portion of the upper end which is first filled, or the mold may be rotated on its vertical axis. This method forms part of another application for patent.

Fig. 3 shows another mode of making the article. In it the wires *a* are stretched in a mold, *g*, which is also to be water-cooled, with glass-tubes *b* upon them. The cast-iron is poured in through a pouring-gate, *h*. The mold *g* may be of any desired form, and differs from the mold *d* in principle, in that it does not have a movable bottom, and that the article cannot exceed in length the length of the mold. This article has the wires completely insulated by the glass tubes, and the cast-iron casing not only surrounds the whole bunch of wires, but penetrates and fills the interstices between the same. The molten iron softens and partially fuses the outer surface of the tube or tubes, so that the glass adheres to the iron when set, and the two become united and substantially integral. The structure of the cast-iron is such that this union is properly effected.

The advantages of my improved article are that the glass insulating tubes are preserved from fracture, that the cast-iron sets in and around and forms a union therewith, that the article can be molded in any shape, that any desired number of wires can be used, that it is

firm and strong structure, easily and cheaply made, completely impervious to moisture, and adapted to general and extensive use for underground-telegraph purposes.

5 What I claim as my invention, and desire to secure by Letters Patent, is—

A telegraph wire or wires surrounded with a glass insulating layer or casing, and an outer enveloping casing of cast-iron united to the

glass, substantially as and for the purposes described.

In testimony whereof I have hereunto set my hand.

WILLIAM H. MAXWELL.

Witnesses:

T. B. KERR,  
J. K. SMITH.

Correction of Letters Patent No. 243,283

It is hereby certified that in Letters Patent No. 243,283, granted June 21, 1881, upon the application of William H. Maxwell, for an improvement in "Insulated Telegraph-Wires," the name of the assignee of two-thirds interest was erroneously written and printed therein "A. S. Tompkinson" instead of "A. S. Tomkinson;" that the correct name is A. S. Tomkinson; that the proper corrections have been made in the files and records pertaining to the case in the Patent Office, and are hereby made in said Letters Patent.

Signed, countersigned, and sealed this 28th day of June, A. D. 1881.

[SEAL.]

A. BELL,  
*Acting Secretary of the Interior.*

Countersigned:

E. M. MARBLE,  
*Commissioner of Patents.*